

**UNITED STATES PATENT OFFICE.**

GLEN LENARDO WILLIAMS, OF NEW YORK, N. Y., ASSIGNOR, BY MESNE ASSIGNMENTS, TO HENRY WALTON CAMPBELL, OF DETROIT, MICHIGAN.

## PROCESS OF ELECTRICALLY DEPOSITING ALUMINIUM

1,351,144.

Specification of Letters Patent. Patented Aug. 31, 1920

No Drawing.

Application filed March 11, 1918. Serial No. 221,736.

*To all whom it may concern:*

Be it known that I, GLEN LENARDO WILLIAMS, a citizen of the United States, residing at New York city, in the county of New York, State of New York, have invented certain new and useful Improvements in Processes of Electrically Depositing Aluminium, of which the following is a specification.

10 This invention relates to a process of producing aluminium from a solution of a compound thereof in a normally liquid electrolyte by the action of electricity and has for its object the production of aluminium in a  
15 direct and economical manner from normally liquid or liquefied substances without the necessity of utilizing a fused electrolyte or vehicle therefor as employed hitherto and it comprises liquefying or dis-  
20 solving an aluminium compound such as aluminium sulfate by or in liquid sulfuric acid of substantially anhydrous character such a substance comprising sulfuric acid containing free sulfuric anhydrid  
25 commonly known as "oleum" containing approximately 85% of sulfuric anhydrid ( $\text{SO}_3$ ) and which readily dissolves 10% of aluminium sulfate, and exposing the aluminium sulfate therein to an electrolysis  
30 preferably employing a current of approximately 3 volts with a cathode of aluminium and an anode of graphite and adding fresh aluminium sulfate or substance capable of forming the same such as alu-  
35 minium oxid or hydroxid to the sulfuric acid as it becomes depleted of aluminium by electrolysis.

As an example of the process and manner in which the same is carried out, the production of aluminium from its sulfate by electrolysis will be taken.

A suitable electrolytic bath or electrolytic vehicle is provided such as the substance commonly known as "oleum" comprising anhydrous sulfuric acid containing sulfuric anhydrid in which is suspended electrodes, the cathode of which comprises aluminium and the anode of which comprises graphite.

50 and the anode of which comprises graphite. To this "oleum" or electrolyte vehicle, comprising substantially sulfuric acid containing 85% of sulfuric anhydrid ( $\text{SO}_3$ ), is primarily added and dissolved therein

aluminium sulfate which is decomposed by the electric current depositing aluminium at the cathode and generating sulfuric anhydrid at the anode which sulfuric anhydrid dissolves in the "oleum" electrolyte vehicle. 55

As the "oleum" vehicle becomes depleted of aluminium by its deposition through electrolysis, aluminium hydroxid or hydrated oxid is added to the "oleum" electrolytic vehicle from time to time to supply a fresh aluminium compound as electrolyte, and which aluminium hydroxid or hydrated oxid is immediately seized by the sulfuric anhydrid present in the "oleum" converting it into new and fresh aluminium sulfate in accordance with the following chemical formula or equation:



In this manner aluminium may be deposited continuously from its solution as a sulfate by electrolysis while in the electrolyte vehicle "oleum" 75

The aluminium sulfate electrolyte while in its solution in "oleum" reduces the electrical resistance so that its electrolysis may be carried on at a voltage at which "oleum" <sup>80</sup> per se would be too highly resistant to allow the transmission of the electric current so that the aluminium sulfate may be electrolytically decomposed or disassociated at a voltage below that at which the "oleum" <sup>85</sup> electrolyte vehicle or solvent is electrolytically affected so that if the tension of the current is maintained at substantially three volts, the aluminium compound is only decomposed to the exclusion of the "oleum" <sup>90</sup> so long as any aluminium compound such as aluminium sulfate is contained in the electrolyte solvent of vehicle "oleum" and the process may be carried on continuously so long as the "oleum" contains or is supplied <sup>95</sup> with aluminium sulfate with an electric current of substantially low voltage in the yielding of aluminium.

There have been many suggestions in the prior art for the electrolytic deposition of aluminium from its compounds while dissolved in an aqueous vehicle, but it has been found that instead of yielding aluminium at the cathode, such aluminium as would be deposited at that point becomes immediately 105

oxidized by the water present, and converted into aluminium hydroxid or hydrated oxid which then immediately dissolves in the solution through the solvent action of 5 the aqueous acid or alkaline electrolyte vehicle and for this reason such processes have not been commercially adaptable.

In the present case it will be seen that the acid electrolyte vehicle "oleum" has no free 10 water to act as a preliminary oxidant whereby the aluminium deposited as metal may be converted into an aluminium compound soluble in the acid, and inasmuch as aluminium *per se* is insoluble in "oleum" it may be deposited electrolytically from a solution of 15 its compound therein, and not be re-dissolved after it is deposited.

It is advisable in order to facilitate the 20 solution or liquefaction of the aluminium compound electrolyte such as aluminium sulfate in the "oleum" vehicle, reduce the electrical resistance of the composition and obtain larger yields in shorter time than the liquid electrolyte and its vehicle be heated 25 to a temperature of 100 degrees C. or to a point at which free water would be ordinarily evolved and dissipated.

Having now described my invention what I claim is:

30 1. The process of producing aluminium which comprises electrolyzing an aluminium compound while dissolved in a normally liquid anhydrous vehicle inert to aluminium and of higher electrical resistance than the aluminium compound to be electrolyzed.

40 2. The process of producing aluminium which comprises electrolyzing an aluminium compound while dissolved in a normally liquid anhydrous acid vehicle inert to aluminium to be electrolyzed.

45 3. The process of producing aluminium which comprises electrolyzing an aluminium compound while dissolved in a normally liquid anhydrous sulfuric acid vehicle inert to aluminium and of higher electrical resistance than the aluminium compound to be electrolyzed.

50 4. The process of producing aluminium which comprises electrolyzing an aluminium compound while dissolved in "oleum".

55 5. The process of producing aluminium which comprises electrolyzing an aluminium sulfate while dissolved in a normally liquid anhydrous vehicle inert to aluminium and of higher electrical resistance than the aluminium sulfate to be electrolyzed.

60 6. The process of producing aluminium which comprises electrolyzing an aluminium sulfate while dissolved in a normally liquid anhydrous acid vehicle inert to aluminium sulfate to be electrolyzed.

65 7. The process of producing aluminium which comprises electrolyzing an aluminium sulfate while dissolved in a normally liquid anhydrous sulfuric acid vehicle inert to

aluminium and of higher electrical resistance than the aluminium sulfate to be electrolyzed.

8. The process of producing aluminium which comprises electrolyzing an aluminium sulfate while dissolved in "oleum".

9. The process of producing aluminium which comprises electrolyzing an aluminium compound while dissolved in a normally liquid anhydrous vehicle inert to aluminium and of higher electrical resistance than the aluminium compound to be electrolyzed while in a heated condition.

10. The process of producing aluminium which comprises electrolyzing an aluminium compound while dissolved in a normally liquid anhydrous acid vehicle inert to aluminium to be electrolyzed while in a heated condition.

11. The process of producing aluminium which comprises electrolyzing an aluminium compound while dissolved in a normally liquid anhydrous sulfuric acid vehicle inert to aluminium and of higher electrical resistance than the aluminium compound to be electrolyzed, while in a heated condition.

12. The process of producing aluminium which comprises electrolyzing an aluminium sulfate while dissolved in "oleum" while in a heated condition.

13. The process of producing aluminium which comprises electrolyzing an aluminium sulfate while dissolved in a normally liquid anhydrous vehicle inert to aluminium and of higher electrical resistance than the aluminium sulfate to be electrolyzed while in a heated condition.

14. The process of producing aluminium which comprises electrolyzing an aluminium sulfate while dissolved in a normally liquid anhydrous acid vehicle inert to aluminium sulfate to be electrolyzed while in a heated condition.

15. The process of producing aluminium which comprises electrolyzing an aluminium sulfate while dissolved in a normally liquid anhydrous sulfuric acid vehicle inert to aluminium and of higher electrical resistance than the aluminium sulfate to be electrolyzed while in a heated condition.

16. The process of producing aluminium which comprises electrolyzing an aluminium sulfate while dissolved in "oleum" while in a heated condition.

17. In the process of electrolytically depositing aluminium from a normally liquid electrolyte, the step which comprises supplying the aluminium compound to be electrolyzed from time to time as the liquid vehicle becomes depleted thereof by electrolysis.

18. In the process of producing aluminium from a normally liquid electrolyte, the step which comprises producing the aluminium compound to be electrolyzed within the liquid electrolytic vehicle by supplying

80

85

90

95

100

105

110

115

120

125

130

thereto from time to time an aluminium compound capable of reacting with a constituent or constituents of the vehicle to produce the compound to be electrolyzed as the liquid vehicle becomes depleted, of the aluminium compound product, by electrolysis.

19. The process of producing aluminium which comprises supplying aluminium oxid or hydroxid to "oleum" electrolyzing the product produced thereby therein and add-

ing more aluminium oxid or hydroxid as the "oleum" is depleted of aluminium by electrolysis.

In testimony whereof I affix my signature in the presence of two witnesses.

GLEN LENARDO WILLIAMS [L. S.]

Witnesses:

PAUL R. NEWMAN,  
WILHELMINA M. LOTZ.